

1

2,701,238

SILVER PROTECTING CLOTH AND PROCESS OF  
MAKING THE SAMEAdolph Renold, Springdale, Conn., assignor to Bates  
Manufacturing Company, a corporation of MaineNo Drawing. Application March 11, 1952,  
Serial No. 276,065

26 Claims. (Cl. 252—192)

This invention relates to a process for preparing silver protecting cloth and to a composition for use in this process and, more particularly, to processes for applying water-insoluble silver salts to textiles which avoid the necessity of precipitating such salts in situ in the textile, and to compositions for use in such processes, and to the products thereof.

Silver protecting cloth has come into wide use as a wrapper for silver to prevent it from tarnishing. The most desirable tarnish-proofing agents for silver appear to be silver salts.

The Grinnell Jones U. S. Patent No. 1,766,646, dated June 24, 1930, describes silver protecting cloths in which silver salts are the tarnish-proofing agents. According to the disclosure of this patent, silver salts are particularly desirable, inasmuch as they react quickly and completely with hydrogen sulfide and the like sulfur-containing gases in much the same manner as silver itself to produce an insoluble silver sulfide. In this way, such gases are kept from reaching the silver articles wrapped in the cloth.

In the process described in the Grinnell Jones patent, the cloth is first impregnated with a solution of a soluble silver salt, such as silver nitrate, and squeezed to remove the excess of silver nitrate solution. Then without drying the cloth a hot alkaline solution of sodium carbonate is applied thereto, causing the silver to be precipitated on and in the cotton fibers as a solid insoluble adherent compound of silver. The cloth then is rapidly washed with water to remove all excess alkali and other soluble substances. This process, although described using silver nitrate and sodium carbonate as illustrative, is in fact applicable to the use of any soluble silver salt initially with the formation of any insoluble silver salt by appropriate reaction with a second soluble salt, as indicated by Grinnell Jones. In fact, the disclosure and the claims of this patent broadly cover any silver constituent in a combination or condition which will combine with the tarnishing gases in the atmosphere accessible to the silverware wrapped in the cloth. Grinnell Jones also indicates that the material impregnated with the insoluble silver salt in finely divided form may be washed without loss of material and presents a very large surface of silver compound for contact with the tarnishing gases.

This procedure of forming the insoluble silver salt in situ on the cloth has the disadvantage that there are present soluble salts which fail to react or are formed as a by-product of the reaction. Silver plate may become damaged through electrolytic action if a soluble salt comes into contact therewith. Therefore, it is necessary to remove any residual soluble salts by careful washing, but usually it is impossible to remove all of the soluble salts, and in consequence, they are deposited on the cloth along with the insoluble silver salt when the cloth is dried. Washing presents the additional objection that some of the insoluble silver salt may be washed out mechanically, as well as the soluble material.

Although the product produced in accordance with the process of the Grinnell Jones patent has been recognized as very effective from the standpoint of protecting silver, attempts have been made to modify the process and thus overcome difficulties which it presents.

One improvement noted in the literature on the method patented by Grinnell Jones appears in U. S. Patent No. 2,003,333 to Kenneth H. Barnard and Henry F. Kane. These investigators point out that the Jones process produces a brown product whose color is so strong as to overpower other dyes. This difficulty is overcome by the use

2

of silver ferrocyanide; precipitating it in situ in the cloth by interaction of two solutions in a process very similar to Grinnell Jones', employing yellow prussiate of soda in place of the sodium carbonate mentioned by Grinnell Jones. A colloid is present in the solution in order to cause the formation of a finely divided precipitate. The precipitation is carried out in a precipitating tank or "jigger" in the presence of the cloth, which has previously been impregnated with the silver nitrate. It is evident that this development is a specific application of the Grinnell Jones process to different silver salts and with the added presence of a colloid. The product is a cloth impregnated with a silver salt formed in situ thereon.

Another modification of the Grinnell Jones process, which likewise results in the formation of a silver protecting cloth impregnated with an insoluble silver salt, is described in Patent No. 2,136,483 to Kenneth H. Barnard and Arthur F. McLean, dated November 15, 1938. The solutions are reacted *au dehors* the fabric in this process, and the precipitate of insoluble silver salt is dissolved by addition of ammonia. This solution then is applied to the textile cloth and the cloth is dried, whereupon the ammonia evaporates and the insoluble silver salt is precipitated. This method has the disadvantage of requiring the use of large quantities of ammonia, which presents a handling and recovery hazard due to the ammonia's unpleasant odor and toxicity. Moreover the solutions are not appreciably less alkaline than the sodium carbonate solutions employed by Grinnell Jones.

Soluble salts are precipitated with the silver salt on the fabric, and must be washed out by the same troublesome washing procedures described by Grinnell Jones. Also, the silver salt precipitated on the cloth is not bound thereto in any way, except as the precipitating procedure may effect the extent to which the particles are within the fibers of the cloth, and the cloth has a tendency to dust, just as in the case of the Grinnell Jones product.

Another modification of the Grinnell Jones process is described in Patent No. 2,480,930 to Elwood C. Jackson and Tully H. Babb, dated September 6, 1949. Jackson and Babb point out that the process of the Barnard et al. Patent No. 2,003,333 indeed has the disadvantage of requiring two steps, and the supplemental difficulty that silver salts present in the cloth may dissolve out in the second bath and precipitate in the solution instead of on the fabric. In order to avoid this, Jackson and Babb propose to precipitate the silver ferrocyanide *au dehors* the cloth as in the Barnard and McLean process and apply the solution containing the finely divided precipitate to the cloth. The solution contains locust bean gum, in order to assure the formation of a finely divided precipitate. However, these investigators admit that the final mixture which is applied to the cloth contains silver ferrocyanide and sodium nitrate, and it is evident in consequence that when the cloth is dried it may contain appreciable quantities of soluble sodium nitrate, which are difficult to remove by washing.

The instant invention provides a process and composition useful in producing silver protecting cloth which avoids the difficulties of all of the prior processes described above in that soluble salts are never present and therefore need not be removed from the treated cloth by special procedures. The soluble salts are eliminated by forming a dispersion comprising finely divided water-insoluble silver salt starting with the water insoluble silver salt rather than by forming the insoluble silver salt by reaction of two soluble salts as in the Grinnell Jones process and the Barnard et al. and Jackson et al. processes following it.

In one preferred embodiment, this dispersion contains a binder which adheres the insoluble silver salt to the cloth, and overcomes the dusting difficulties attributable to nonbinder-containing products heretofore available. There is obtainable with this dispersion a textile product having a water-insoluble silver salt distributed thereon and adhered thereto by the binder.

Heretofore it has been thought impossible to prepare aqueous dispersions of water-insoluble silver salts except by precipitation of the silver salt in situ, desirably in the presence of a colloid. In accordance with the instant invention, however, a concentrated dispersion contain-

ing a finely divided water-insoluble silver salt is formed by dispersing the insoluble silver salt in a grinding liquid in the presence of a filler which can function both as a grinding aid in reducing the silver salt to a dispersible particle size and as a protective colloid or dispersing agent for the silver salt. This dispersion can be diluted with water to form an aqueous dispersion of a solids content suitable for direct application to a textile to produce a silver protecting cloth without applying at the same time any of the soluble by-product salts which have led to difficulties heretofore.

The invention makes possible the treatment of textiles with any water-insoluble silver compound, including the oxide and salts of inorganic and organic acids. Typical water-insoluble silver salts coming within the scope of the invention are silver iodate, silver pyrophosphate, silver carbonate, silver palmitate, silver stearate, silver metaphosphate, silver orthophosphate, silver ferricyanide and silver ferrocyanide.

The filler employed in conjunction with the silver salt has a dual function. It assists in reducing the silver salt to a finely-divided particle size and thus serves as a grinding agent. In addition, in the presence of water, the filler takes on the character of a protective colloid or dispersing agent, and assists in dispersing the finely divided silver salt in the aqueous medium and maintaining it in dispersed form. Materials which have been found satisfactory as fillers include natural starches, such as corn, sago, maize, cassava, arrowroot, wheat and potato starches, and modified and incompletely hydrolyzed starches, such as the dextrines derived from cassava, corn, potato, sago and wheat starches, and converted or modified corn starch.

The silver salt can be reduced to the desirable finely-divided form by grinding it with the filler in a conventional ball, roll or pebble mill. A three-roll mill can be used, for example, with the rolls set at less than 0.0001 inch clearance. Those skilled in the art know other suitable grinding methods and apparatus. In general, it may be stated that equipment useful for reducing pigments to a finely-divided form for dispersion in paints can be employed in the instant invention.

It is desirable to have a grinding liquid present to assist the grinding and to serve as the dispersing medium for the silver salt. Water is quite satisfactory for this purpose and is preferable because it also is the preferred dispersant for the diluted dispersion which is applied to the textile. A grinding oil may be more effective than water in preparing dispersions of higher solids contents. Liquid detergents such as any of those listed herein-after and especially nonionic detergents, e. g., alkyl aryl polyether alcohols such as Triton X-100 (polyethylene glycol-octyl alcohol reaction product) can also be used as the grinding liquid. Other suitable liquid detergents are polyethylene glycol esters of rosins and polyethylene glycol ethers of alkylated phenols as exemplified by the Hercules synthetics B-48, B-79 and B-97.

Grinding oils are well known to those skilled in the paint art, and any of these known oils can be employed. For example, modified linseed oils, as exemplified by Trimol No. 80, and soya oil-maleic anhydride reaction products, as exemplified by Soya Trimol No. 4, and mineral oil have been found satisfactory.

From 0.5 to 2 parts of filler per part of silver salt by weight make possible the production of a stable, concentrated dispersion. From 0.5 to 2 parts of grinding liquid, which may be water, grinding oil or a liquid detergent, per part of silver salt should also be used. These ranges represent satisfactory minimum proportions. Optimum proportions are 1 part silver salt to 1.7 parts grinding liquid to 1 part filler.

Only as much filler and grinding liquid as is necessary to disperse the silver salt should be used. Although the stated proportions of filler and grinding liquid to silver salt may be greater than those stated, larger quantities of those materials are not necessary. In fact, excessively large quantities are to be avoided, for the silver salt may be enveloped in filler and/or grinding liquid, if the latter is not volatile, after deposition thereof on the textile, and hydrogen sulfide then would be kept from reaching and reacting with the silver salt, thus defeating the purpose of the composition.

To the concentrated dispersion there can be added from 0.5 to 1 part of a protective colloid per part of silver salt. This component is not essential and the proportions

thereof are not critical, but its presence assist in making a smooth dispersion which remains suitable for long periods. Protective colloids which have given satisfactory results in this respect are methyl cellulose and sodium carboxymethylcellulose.

When water and like volatile liquids are used as the grinding liquid, no difficulties are encountered, either in the grinding procedure or in the preparation of the aqueous dispersion from the concentrate, and textiles treated with such dispersions show excellent protection to silver-ware. However, some dusting of silver salt may occur.

To avoid this, it is especially desirable to include a binding agent in dispersions in which water or other volatile liquid is employed as the grinding liquid, although a binder can be used with advantage when non-volatile grinding liquids are employed as well. This material can be used at a concentration within the range from 0 to 45%. Modified alkyd resins are preferred binding agents. Suitable binders are: Trimol No. 80 (linseed oil, maleic anhydride reaction product), Trimol No. 4 (soya oil maleic anhydride reaction product), Rezyl 387-5 (short oil oxidizing type soya modified alkyd resin dissolved in xylene), Aroplaz 1273 (vegetable drying oil-modified phthalic anhydride-pentaerythritol alkyd resin), and Aroflat 3050-P-40 (vegetable drying oil-modified pentaerythritol-alpha, beta-ethylenically unsaturated dibasic acid alkyd-resin).

In some instances, a material which is useful as a grinding oil will also be useful as a binder. For example, some soya oil-maleic anhydride reaction products have binding properties. When the grinding oil has the properties of a binder, it is not necessary to include a supplemental binder in the dispersion.

The concentrated dispersion prepared as described above containing silver salt, filler and grinding medium may have too high a solids concentration for convenient application to a textile. In this event it is preferable to dilute the concentrated dispersion with water. The dispersion should be of such a solids content that it will not be viscous and when applied to the cloth at a 50 to 135% wet pickup by weight, there will be provided from 0.2 to 2.5% silver metal by weight on the cloth. More than this may be applied if desired, but it is not necessary. In order to preserve the hand of the cloth, it is desirable to keep the total solids applied to the cloth below 10% and usually in the range from about 1% to about 7% by weight of the cloth. Usually these conditions are adequately met by a dispersion having a solids content of not over 12% by weight. Such dispersions are not very viscous and give a good total penetration throughout the cloth.

Dilution of the concentrated dispersion with water can be effected as follows: The concentrated dispersion is poured slowly into a vessel containing approximately one-third of the water required to produce a dispersion of the desired solids content, at room temperature, while agitating violently and with injection of live steam. In the course of addition of the concentrated dispersion, the temperature of the water is increased to nearly the boiling point, i. e., between 190° to 200° F., and the diluted dispersion is held at a temperature within this range for about five minutes which allows the filler to assume the character of a protective colloid and maintain the silver salt in dispersed form in the aqueous medium. The dispersion is then quickly cooled to room temperature.

Other dilution procedures may be employed, but it is important to avoid "breaking" the emulsion in which the silver salt is held in suspension.

In order to avoid damage to the textile, it is usually desirable that the diluted aqueous dispersion which is applied thereto not be acid. On the other hand, at too alkaline a pH the silver salt may be hydrolyzed. Therefore, it is preferable that the pH of the diluted dispersion lie within the range from about 7 to about 8. Since the concentrated dispersion containing the ingredients set forth above usually has a pH slightly on the acid side, in order to bring the pH of the concentrated and of diluted dispersions prepared therefrom to within the range set forth, it is necessary to add an alkaline material to either dispersion. The alkaline material should be volatile, so that it will be removed when the fabric which has been padded with the dispersion is dried. Satisfactory volatile alkaline materials are ammonium hydroxide and the organic amines of lower molecular weight, such as morpholine, ethylamine, propylamine,

butylamine, diisopropylamine, pyrrolidine and diethylamine.

To facilitate wetting of the textile by the dispersion a small amount of a wetting agent or detergent, usually not over approximately 1% by weight, can be added to either the concentrated or diluted dispersion. Non-ionic wetting agents and detergents are preferred, such as alkylated aryl polyether alcohols, e. g., polyethylene glycol-octyl alcohol reaction products, as exemplified by Triton X-100, polyethylene glycol esters of rosin, sorbitan monolaurate, palmitate and stearate, polyoxyethylene derivatives (the Tweens), polyoxyethylene stearate, caprate, laurate and oleate, ethylene oxide condensates with fatty alcohols and fatty acids, glycerol monostearate, and fatty acid-amine ester condensates. A wide variety of nonionic wetting agents are known to those skilled in the art and therefore further details need not be set forth herein. Anionic and cationic wetting agents also may be used, if desired, with good results; however, they must not be reactive with silver. For this reason, they must not contain chloride ion, or sulfur.

Additional optional materials include antifoamers such as mixtures of paraffin wax and glycerol monostearate and silicone resins, and driers such as cobalt and lead naphthenates, which can also be added as desired.

Some grinding oils have strong odors and may impart an undesirable odor to the silver protecting cloth. This disadvantage may be overcome by incorporating a small quantity of the order of 0.5 to 1% of a deodorant oil or perfume in the concentrated or diluted dispersion. Some drying oils and modified alkyd resins are odorless and therefore do not present this problem. However, when modified alkyd resins are employed it is desirable to incorporate additional quantities of organic solvents to facilitate preparation of the dispersion, and cobalt or lead naphthenate driers should also be added.

As stated, the concentration of the diluted dispersion with respect to silver and the wet pick-up of the cloth are adjusted so that there will be provided at least 0.2% silver, calculated as the metal, by weight of the textile. Obviously, in meeting this requirement, the proportions of silver compound present in the diluted aqueous dispersion will be varied in relation to the percentage of silver in the silver salt employed. It will be evident that the quantity of silver stearate required will be larger than that of silver carbonate or silver pyrophosphate, because of the lower proportion of silver in silver stearate.

The following table shows in terms of silver pyrophosphate the composition of various diluted aqueous dispersions containing a binder which can be prepared, using water, binder and wetting agent as the grinding liquids. The amount of silver pyrophosphate can, by calculation, as those skilled in the art are aware, be changed to accommodate other silver compounds from a knowledge of the silver content of the other compounds, and by increasing or decreasing the amounts of filler, binder and other ingredients accordingly in accord with the recommended proportions of these materials to silver compound heretofore set forth.

TABLE I

|                                                    |                 |           |
|----------------------------------------------------|-----------------|-----------|
| Silver pyrophosphate                               | per cent solids | 16.2-43.7 |
| Filler                                             | do              | 16.5-35.2 |
| Binder                                             | do              | 0.0-45.3  |
| Alkaline material                                  | do              | 0.1-4.3   |
| Wetting agent                                      | do              | 1.3-33.0  |
| Parts of water to each part of above concentration |                 | 7.3-179   |

The preferred application procedure consists in dipping the dyed cloth in the aqueous dispersion, with subsequent squeezing and drying. If flannel is used, the cloth can be given a light renapping for a fuller hand and better appearance.

Conventional padding equipment is employed in applying the diluted dispersion to the textile, and the padding is carried out in the usual manner well known to those skilled in the art. The padded cloth is dried at temperatures which will not damage the textile, depending of course upon the nature of the textile, and is then ready for use.

The following examples are given to further illustrate the invention:

## Example 1

A concentrated dispersion of silver pyrophosphate in a grinding oil (Soya Trimol No. 4) was prepared by grinding a mix having the following composition:

|                                                                       | Parts |
|-----------------------------------------------------------------------|-------|
| Silver pyrophosphate                                                  | 100   |
| Converted corn starch                                                 | 80    |
| Soya Trimol No. 4 (liquid soya oil-maleic anhydride reaction product) | 180   |
| White dextrose                                                        | 20    |

by three passes in a three-roll mill with the clearance set at 0.0001 inch.

The concentrate was poured slowly into a tank containing about one-third of the water needed to dilute the concentrate to a dispersion having a 2.46% silver pyrophosphate content. This was done while the water, at room temperature, was agitated violently by injecting live steam with stirring. The temperature was brought nearly to boiling and held there for about 5 minutes. The steam was then turned off and a quantity of cracked ice equal to about one-third the total weight of water was added with stirring. Tap water at room temperature was then added to bring the dispersion to the correct volume. Morpholine, perfume, methyl cellulose and Triton X-100 were added to form a final dispersion of pH 7 having the following composition:

|                                                                                                        | Percent |
|--------------------------------------------------------------------------------------------------------|---------|
| Silver pyrophosphate                                                                                   | 2.46    |
| White dextrose                                                                                         | 0.50    |
| Converted corn starch                                                                                  | 1.96    |
| Soya Trimol No. 4 (soya oil-maleic anhydride reaction product)                                         | 3.30    |
| Morpholine                                                                                             | 0.32    |
| Perfume                                                                                                | 0.20    |
| Methyl cellulose                                                                                       | 1.35    |
| Triton X-100 (condensation product of octyl phenol and polyethylene glycol (8-12 mols ethylene oxide)) | 2.00    |
| Water                                                                                                  | 87.94   |

This dispersion was padded on maroon flannel to a 50% wet pick-up by weight and dried, thus depositing 1.23% silver pyrophosphate by weight on the cloth, the cloth then was given a light renapping. The flannel had good hydrogen sulfide absorbency and a good hand. Little change in color of the flannel was observed.

## Example 2

Silver pyrophosphate was ground with modified starch, white dextrose and Rezyl 387-5 (a short oil oxidizing type pure alkyd resin dissolved in xylene) morpholine and Triton X-100 to prepare a concentrated dispersion of the silver pyrophosphate of the following composition, in which the alkyd resin and xylene serve as the grinding medium:

|                                                        | Percent |
|--------------------------------------------------------|---------|
| Silver pyrophosphate                                   | 33.6    |
| White dextrose                                         | 4.9     |
| Modified corn starch                                   | 19.5    |
| Rezyl 387-5 (modified alkyd resin dissolved in xylene) | 27.5    |
| Xylene                                                 | 3.1     |
| Morpholine                                             | 0.7     |
| Triton X-100                                           | 10.7    |

One part of the resulting concentrate was diluted with 12 parts of water as indicated in Example 1. To this the customary amounts of cobalt and lead driers and a trace of antifoaming agent were added (silicone resin antifoamer). This dispersion, which had a pH of about 7, was then padded on a flannel to a 50% wet pick-up, by weight and dried. The cloth was given a light renapping, after which it displayed a good hand and excellent hydrogen sulfide absorption.

## Example 3

A concentrated dispersion was prepared of silver pyrophosphate in Triton X-100 having the following composition, using the three-roll mill of Example 1:

|                      | Percent |
|----------------------|---------|
| Silver pyrophosphate | 44.0    |
| Modified corn starch | 21.9    |
| Morpholine           | 1.2     |
| Triton X-100         | 32.9    |

This composition was dispersed in water using the procedure described in Example 1, and to this dispersion was added an antifoaming agent (silicone resin antifoamer) resulting in a dispersion of the following composition:

|                                               | Percent |
|-----------------------------------------------|---------|
| Silver pyrophosphate                          | 2.00    |
| Modified corn starch                          | 1.00    |
| Morpholine                                    | 0.005   |
| Triton X-100                                  | 1.50    |
| Antifoaming agent (silicone resin antifoamer) | 0.005   |
| Water                                         | 95.44   |
| pH 7 to 8                                     |         |

A second dispersion was prepared which was identical with the above, with the exception that 1.5% of an alkyd resin was added. This dispersion had the following composition:

|                                               | Percent |
|-----------------------------------------------|---------|
| Silver pyrophosphate                          | 2.00    |
| Modified corn starch                          | 1.00    |
| Morpholine                                    | 0.005   |
| Triton X-100                                  | 1.50    |
| Rezyl 387-5                                   | 1.50    |
| 6% Cobalt drier                               | 0.012   |
| Antifoaming agent (silicone resin antifoamer) | 0.005   |
| Water                                         | 93.928  |
| pH 7 to 8                                     |         |

Each of these dispersions was padded on a flannel cloth to a 110% wet pick-up by weight and dried. The cloths after renapping in each case had a good hand and showed excellent hydrogen sulfide absorption, giving good protection to silverware enclosed therein. The cloth padded with the composition containing alkyd resin (Rezyl 387-5) showed no tendency to dust.

#### Example 4

A concentrated dispersion was prepared of silver pyrophosphate in water having the following composition:

|                      | Percent |
|----------------------|---------|
| Silver pyrophosphate | 48.1    |
| Modified corn starch | 24.1    |
| Morpholine           | 1.9     |
| Triton X-100         | 1.9     |
| Water                | 24.0    |

This concentrate was dispersed in water as described in Example 1 to produce a dispersion to which antifoam was added, having the following composition:

|                                               | Percent |
|-----------------------------------------------|---------|
| Silver pyrophosphate                          | 2.00    |
| Modified corn starch                          | 1.00    |
| Morpholine                                    | 0.079   |
| Triton X-100                                  | 1.50    |
| Antifoaming agent (silicone resin antifoamer) | 0.005   |
| Water                                         | 95.416  |
| pH 7                                          |         |

A second dispersion was prepared which was identical with the above, but contained 1.5% of an alkyd resin. This dispersion had the following composition:

|                                               | Percent |
|-----------------------------------------------|---------|
| Silver pyrophosphate                          | 2.00    |
| Modified corn starch                          | 1.00    |
| Morpholine                                    | 0.079   |
| Triton X-100                                  | 1.50    |
| Rezyl 387-5                                   | 1.50    |
| 6% Cobalt drier                               | 0.012   |
| Antifoaming agent (silicone resin antifoamer) | 0.005   |
| Water                                         | 93.904  |
| pH 7 to 8                                     |         |

Each of these dispersions was padded on a flannel cloth to a 110% wet pick-up by weight and dried, after which the cloth was given a light renapping. The cloths had a good hand and gave good protection to silverware wrapped therein. The cloth padded with the dispersion which contained alkyd resin showed no tendency to dust silver salt.

#### Example 5

A concentrated dispersion was prepared using mineral oil as the grinding liquid and initial dispersant, and having the following composition:

|                      | Percent |
|----------------------|---------|
| Silver pyrophosphate | 34.7    |
| Modified corn starch | 17.4    |
| Morpholine           | 1.3     |
| Triton X-100         | 1.3     |
| Mineral oil          | 45.3    |

This concentrate was diluted with water as described in Example 1 and to the resulting dispersion an antifoaming agent was added. The dispersion had the following composition:

|                                               | Percent |
|-----------------------------------------------|---------|
| Silver pyrophosphate                          | 2.00    |
| Modified corn starch                          | 1.00    |
| Morpholine                                    | 0.075   |
| Triton X-100                                  | 0.075   |
| Antifoaming agent (silicone resin antifoamer) | 0.005   |
| Mineral oil                                   | 2.615   |
| Water                                         | 94.230  |

This dispersion was padded on a flannel cloth to a 110% wet pick-up by weight and then dried. The cloth after renapping had a good hand and gave excellent protection to silverware wrapped therein.

#### Example 6

A concentrated dispersion was prepared of silver stearate in alkyd resin, xylene and liquid detergent (Triton X-100) using the three-roll mill of Example 1 and having the following composition:

|                      | Percent |
|----------------------|---------|
| Silver stearate      | 35.2    |
| Modified corn starch | 25.8    |
| Morpholine           | 0.5     |
| Triton X-100         | 7.9     |
| Rezyl 387-5          | 21.7    |
| Xylene               | 8.9     |

This concentrate was dispersed in water as described in Example 1, and to the resulting dispersion a solution of a modified alkyd resin in xylene, an antifoaming agent and cobalt drier were added to produce the following dispersion:

|                                               | Percent |
|-----------------------------------------------|---------|
| Silver Stearate                               | 2.46    |
| Modified corn starch                          | 1.81    |
| Rezyl solution 387-5                          | 1.52    |
| Xylene                                        | 0.62    |
| Morpholine                                    | 0.03    |
| Triton X-100                                  | 0.55    |
| 6% cobalt drier                               | 0.012   |
| Antifoaming agent (silicone resin antifoamer) | 0.005   |
| Water                                         | 92.993  |
| pH 7                                          |         |

This dispersion was padded on a flannel cloth to a 50% wet pick-up by weight. The dry flannel had a good hand and definitely prevented the tarnishing of silverware enclosed therein.

In order to provide a cloth with the long life of a cloth treated with a dispersion containing 2% silver pyrophosphate the silver stearate content of the above dispersion should be increased to about 5.1% due to the smaller per cent of silver contained in silver stearate.

#### Example 7

The following example shows that dispersions having very low concentrations of silver salt can be employed when applied at a wet pick-up of 100% or more. The concentrated dispersions were prepared of silver pyrophosphate in Triton X-100, and then diluted with water as set forth in Example 1. These dispersions had the following composition:

|                      | Percent A | Percent B | Percent C |
|----------------------|-----------|-----------|-----------|
| Silver pyrophosphate | 0.500     | 0.250     | 0.125     |
| Modified corn starch | 0.268     | 0.130     | 0.065     |
| Rezyl 387-5          | 0.148     | 0.074     | 0.037     |
| Toluene              | 0.087     | 0.043     | 0.022     |
| Morpholine           | 0.007     | 0.003     | 0.002     |
| Triton X-100         | 0.107     | 0.054     | 0.027     |
| 6% cobalt drier      | 0.012     | 0.006     | 0.006     |
| Antifoaming agent    | 0.005     | 0.003     | 0.003     |
| Water                | 98.876    | 99.437    | 99.713    |
| pH 7 to 8            |           |           |           |

Each of these dispersions was padded on flannel to a 111% wet pick-up by weight. The cloths were dried and given a light renapping. Dispersion A yielded a treated cloth containing 0.42% silver, by calculation, from the weight of silver salt therein, dispersion B a cloth containing 0.2% silver, by calculation, and dispersion C a cloth containing 0.1% silver, by calculation. The first two cloths gave adequate protection against tarnish to silverware enclosed therein. The cloth obtained from dispersion C did not give good silver protection, the silver becoming tarnished within approximately 4 hours after an exposure of 1 cubic centimeter of hydrogen sulfide per hr., showing that about 0.2% silver is the effective minimum for adequate protection.

*Example 8*

A concentrated dispersion of silver iodate in alkyd resin and liquid detergent (Triton X-100) was prepared having the following composition:

|                      | Percent |
|----------------------|---------|
| Silver iodate        | 33.5    |
| Modified corn starch | 35.2    |
| Rezyl 387-5          | 21.9    |
| Xylene               | 0.9     |
| Morpholine           | 0.5     |
| Triton X-100         | 8.0     |

A portion of this concentrate was dispersed in water in the ratio of 1 part to 11.3 parts of water and a second portion dispersed in water in the ratio of 1 part to 17.1 parts of water as set forth in Example 1.

Each of these dispersions had a pH of about 7, and when padded on flannel cloth to a 50% wet pick-up by weight produced cloths having a good hand and giving excellent protection to silverware wrapped therein.

*Example 9*

A concentrated dispersion of silver carbonate in alkyd resin and liquid detergent (Triton X-100) was prepared having the following composition:

|                      | Percent |
|----------------------|---------|
| Silver carbonate     | 38.7    |
| Modified corn starch | 28.1    |
| Rezyl 387-5          | 24.1    |
| Morpholine           | 0.5     |
| Triton X-100         | 8.6     |

This concentrate was dispersed in water in the ratio of 1 part to 13.3 parts of water. The resulting dispersion, which had a pH of about 7, was padded on a flannel cloth to a 50% wet pick-up by weight, after which the cloth was given a light renapping. The cloth had a good hand and excellent hydrogen sulfide absorption, giving extremely good hydrogen sulfide protection to silverware enclosed therein; with no dusting being evidenced.

*Example 10*

The following is an example of a diluted aqueous dispersion of silver palmitate:

|                                                               | Percent |
|---------------------------------------------------------------|---------|
| Silver palmitate                                              | 1.75    |
| White dextrine                                                | 0.60    |
| Alkali-modified corn starch                                   | 0.60    |
| Trimol No. 80 (linseed oil-maleic anhydride reaction product) | 1.75    |
| Morpholine                                                    | 0.20    |
| Deodorant                                                     | 0.10    |
| Methyl cellulose                                              | 0.66    |
| Triton X-100                                                  | 1.00    |
| Silicone resin antifoaming agent                              | 0.05    |
| Water                                                         | 93.29   |

This dispersion, upon application to a flannel cloth at a 100% pick-up by weight, drying and renapping, produces a silver protecting cloth which shows excellent hydrogen sulfide absorption and gives good protection to silverware enclosed therein.

In the above examples, in many instances a particular liquid or liquid mixture is referred to as the grinding liquid. Actually, however, all of the liquids present in the grinding mix can in a sense be collectively regarded as the grinding medium, since it is very difficult to determine the exact state of the dispersed silver salt when a mixture of liquids is used.

The process of the invention can be applied to textile

fabrics of all kinds. Various modes of preparing the textiles for impregnation can be used, and it will be understood that any such methods as are known to those skilled in the art are contemplated as within the variations of the invention. The process is applicable to textile fabrics in the greige and to dyed textile fabrics. It will be found that as a general rule the color of the dyed fabrics is little affected by the process of the invention, provided the total amount of composition by weight of the fabric does not exceed the amounts recommended herein.

If desired, when greige or bleached fabrics are being treated, pigments may be incorporated in the dispersion or the composition of the invention to produce a colored cloth. In this event, however, it is especially important to employ the minimum quantities required of filler in order to obtain the maximum effect from the pigments incorporated therein.

The following example is illustrative of a pigment containing composition:

*Example 11*

A concentrated dispersion of silver pyrophosphate in a grinding oil (Soya Trimol No. 4) was prepared using a three-roll mill according to the following formulation:

|                                          | Parts |
|------------------------------------------|-------|
| Silver pyrophosphate                     | 100   |
| Modified corn starch                     | 80    |
| White dextrine                           | 20    |
| Soya Trimol No. 4                        | 174.8 |
| Atlantic Red Toner (organic red pigment) | 81.3  |

The concentrate was diluted slowly according to the procedure outlined in Example 1, with the amount of water needed to produce a diluted dispersion having a 1.23% silver pyrophosphate content. Morpholine, methyl cellulose, deodorant and Triton X-100 were added to form a final dispersion of pH 7 having the following composition:

|                             | Per cent |
|-----------------------------|----------|
| Silver pyrophosphate        | 1.23     |
| White dextrine              | 0.25     |
| Alkali-modified corn starch | 0.98     |
| Atlantic Red Toner          | 1.00     |
| Soya Trimol No. 4           | 2.15     |
| Morpholine                  | 0.16     |
| Deodorant                   | 0.10     |
| Methyl cellulose            | 0.75     |
| Triton X-100                | 1.00     |
| Water                       | 92.38    |

This dispersion was padded on a flannel to a 100% wet pick-up by weight and dried, thus depositing 1.23% silver pyrophosphate by weight on the cloth, and the cloth given a light renapping. The flannel had a good red color, excellent hydrogen sulfide absorbency and a good hand.

If a shade other than red is desired, other suitable color pigments can be used, following the same procedure.

It is evident from the above description that only the silver salt, filler and grinding liquid are the essential ingredients of the concentrated dispersion, and that the other components, i. e., the binder, wetting agent, anti-foaming agent, protective colloid, driers, alkaline material, etc. can be added to either the concentrated dispersion or the diluted dispersion, as may prove convenient, or can be omitted entirely.

In many of the examples given the dispersions are designed to be applied to the textile material at a 50% wet pick-up by weight. It will be understood that the concentration of the dispersions can be modified for a 100% wet pick-up by weight merely by cutting the concentrations of the various components in half. This, for example, can be done with the compositions of Examples 1, 2, 6, 8 and 9. On the other hand, by doubling the concentrations of the components in Examples 3, 4, 5, 10 and 11, the wet pick-up can be reduced to 50% by weight. Those skilled in the art will readily perceive that in this way dispersions adapted for any wet pick-up by weight can be prepared.

All proportions and percentages in the specification and claims are by weight.

I claim:

1. A textile-treating composition for producing silver protecting textile material, comprising a water-insoluble

silver compound reactive with hydrogen sulfide and a solid filler-grinding aid selected from the group consisting of natural starches and modified and incompletely hydrolyzed starches in the proportion of at least one-half part filler-grinding aid per part of silver compound but less than will render the silver compound unavailable for reaction with hydrogen sulfide after deposition on a textile, the silver compound and filler-grinding aid being ground and dispersed together in finely-divided form in a drying oil in the proportion of at least one-half part drying oil per part of silver compound, said composition being free from water-soluble salts.

2. A composition in accordance with claim 1 in which the silver compound is silver pyrophosphate.

3. A composition in accordance with claim 1 in which the silver compound is silver stearate.

4. A composition in accordance with claim 1 in which the silver compound is silver carbonate.

5. A composition in accordance with claim 1 in which the silver compound is silver iodate.

6. A composition in accordance with claim 1 in which the drying oil is a soya oil-maleic anhydride reaction product.

7. A composition in accordance with claim 1 which also includes a volatile alkali in an amount less than will dissolve the silver compound but sufficient to bring the pH of a dilute aqueous dispersion of the composition to within the range from about 7 to about 8.

8. A composition in accordance with claim 7 in which the alkali is morpholine.

9. A composition in accordance with claim 7 in which the alkali is ammonia.

10. A composition in accordance with claim 1 which includes from one-half to one part, per part of silver compound, of a protective colloid in addition to the filler-grinding aid.

11. A composition in accordance with claim 1 in which the filler-grinding aid is a dextrine.

12. A composition in accordance with claim 1 in which the filler-grinding aid is a natural starch.

13. A composition in accordance with claim 1 which includes up to 45% by weight of the solids content of the composition of a synthetic resinous binder in addition to the filler-grinding aid.

14. A composition in accordance with claim 13 in which the binder is an oil modified alkyd resin.

15. An aqueous textile-treating dispersion for use in producing silver protecting textile material comprising a water-insoluble silver compound reactive with hydrogen sulfide, a solid filler-grinding aid selected from the group consisting of natural starches and modified and incompletely hydrolyzed starches in the proportion of at least one-half part filler-grinding aid per part of silver compound but less than will render the silver compound unavailable for reaction with hydrogen sulfide after deposition on a textile, the silver compound and filler-grinding aid being ground and dispersed together in finely-divided form in a liquid dispersing medium in the proportion of

at least one-half part liquid per part of silver compound, and a resinous binder in an amount up to approximately 45% by weight of the solids content of the dispersion in addition to the filler-grinding aid, said composition being free from water-soluble salts.

16. A dispersion in accordance with claim 15 which includes a volatile alkali in an amount less than will dissolve the silver compound but sufficient to bring the pH to within the range from about 7 to about 8.

17. A dispersion in accordance with claim 15 which includes a wetting agent.

18. A process of preparing silver silver-protecting textile material which comprises applying to the material a dispersion in accordance with claim 15 and then drying the material.

19. A textile material having distributed thereon and adhered thereto a composition comprising a water-insoluble silver compound reactive with hydrogen sulfide and in a condition available for such reaction, and a

20. filler-grinding aid selected from the group consisting of natural starches and modified and incompletely hydrolyzed starches in the proportion of at least one-half part filler-grinding aid per part of silver compound but less than will render the silver compound unavailable for

25. reaction with hydrogen sulfide, the silver compound and filler-grinding aid having been ground and dispersed together in finely-divided form prior to deposition on the textile, and a synthetic resinous binder in an amount up to approximately 45% by weight of the composition,

30. said textile material being free from water-soluble salts.

20. A textile material in accordance with claim 19 in which the silver compound is silver pyrophosphate.

21. A textile material in accordance with claim 19 in which the silver compound is silver stearate.

35. 22. A textile material in accordance with claim 19 in which the silver compound is silver carbonate.

23. A textile material in accordance with claim 19 in which the silver compound is silver iodate.

40. 24. A textile material in accordance with claim 19 in which the binder is an oil modified alkyd resin.

25. A textile material in accordance with claim 19 in which the binder is a soya oil-maleic anhydride reaction product.

45. 26. A composition in accordance with claim 15 in which the binder is an oil-modified alkyd resin.

#### References Cited in the file of this patent

#### UNITED STATES PATENTS

|    |           |          |               |
|----|-----------|----------|---------------|
| 50 | 1,972,323 | Shiraeff | Sept. 4, 1934 |
|    | 2,184,310 | Meigs    | Dec. 26, 1939 |
|    | 2,434,190 | Barnes   | Jan. 6, 1948  |
|    | 2,480,930 | Jackson  | Sept. 6, 1949 |
|    | 2,500,113 | Banks    | Mar. 7, 1950  |
| 55 | 2,527,261 | Hart     | Oct. 24, 1950 |
|    | 2,550,345 | Gray     | Apr. 24, 1951 |
|    | 2,565,418 | Yackel   | Aug. 21, 1951 |
|    | 2,600,719 | Wood     | July 17, 1952 |